

March 13, 1934.

C. A. ALT ET AL

1,951,119

PRODUCTION OF COATED FABRICS

Filed Sept. 22, 1931



Cornelius A. Alt, INVENTORS  
Herman C. Graebner,  
Lancelot Moffett

BY

J. M. Castle Jr.  
ATTORNEY.

## UNITED STATES PATENT OFFICE

1,951,119

## PRODUCTION OF COATED FABRICS

Cornelius A. Alt, Herman C. Graebner, and  
Lancelot Moffett, Newburgh, N. Y., assignors to  
E. I. du Pont de Nemours & Company, Wilming-  
ton, Del., a corporation of Delaware

Application September 22, 1931, Serial No. 564,282

10 Claims. (Cl. 91—68)

This invention relates to the production of coated fabrics, and more particularly, to the production of translucent shade cloth for window shades, and the like, of improved appearance.

5 Shade cloth comprising a fabric coated with a cellulose ester base has been known in the art for a considerable time. Such shade cloth to be satisfactory must be easy to clean, have great resistance to deterioration on exposure, and be 10 durable. Besides such properties, shade cloth must be of satisfactory appearance, that is, it must possess a clearness when viewed by transmitted light, have a uniformity of translucency, a generally attractive appearance and a so-called 15 smooth feel. These latter properties relate to the so-called "eye" value of the shade cloth, and the present invention is particularly concerned with the production of shade cloth of improved properties relating to "eye" value. Heretofore known 20 shade cloth of this type has been fairly satisfactory as far as wearing qualities are concerned, but the appearance of the cloth leaves considerable room for improvement, particularly with respect to uniformity of translucency and clearness when 25 viewed by transmitted light.

An object of the present invention is to provide a simple and economical method of preparing this type of shade cloth of improved clearness when viewed by transmitted light, of greater uniformity of translucency, of smooth feel, and generally improved appearance. A further object is 30 to provide a method of preparing shade cloth of greater durability. Other objects will be apparent from the description of the invention given 35 hereinafter.

These objects are accomplished according to the present invention by applying a cellulose ester coating composition to both sides of a web of textile fabric, such as sheeting, subjecting the 40 coated web to pressure, for example, running the web through a plate press or pressure rolls, and then applying a cellulose ester composition to both sides of the coated web.

In the single figure of the accompanying drawing is shown a cross sectional view of a piece of shade cloth prepared according to this invention. The web of textile fabric 1 has applied to both sides a cellulose ester coating composition 2 which, as shown in the drawing, is forced into the fabric 50 1, but presents a smooth, uniform, outer surface due to the pressure treatment. Reference numeral 3 denotes the second film of cellulose ester coating composition which is applied to both sides of the coated web after subjecting same to the 55 pressure treatment.

The following examples are given to illustrate specific embodiments of the invention, although it is to be understood that the invention is in no way limited to these specific embodiments:

Example 1.—To the web of sheeting weighing 60 2.7 ounces per square yard and having a thread count of 68x68 is applied on one side from 0.2—0.8, preferably 0.4, ounces of a coating composition as follows, parts being by weight:

|                 | Parts |
|-----------------|-------|
| Cellulose ester | 25-60 |
| Softener        | 15-30 |
| Pigment         | 25-40 |

The preferred composition is as follows:

|                 | Parts |
|-----------------|-------|
| Cellulose ester | 41    |
| Softener        | 20    |
| Pigment         | 39    |

The weights given above and throughout the 75 specification include only the so-called "solids" of the coating composition, that is, they do not include solvents and diluents which may or may not be added, as desired, to obtain a coating composition of the desired viscosity. This coating 80 composition may be applied in one or several coats and by any known means, the conventional doctor knife being the preferred form of apparatus for this coating operation.

A like amount of the coating composition is 85 applied to the other side of the web, which is then, while the coatings thus applied are still in a plastic state, run through a plate press of the type usually employed for embossing, or through pressure rolls. The plates in the press 90 may be smooth or may have a shallow engraving upon them, such as a "Skiver" grain, or the like. The pressure exercised by the plate press or the pressure rolls may be varied widely, but is preferably about 575 pounds per square inch. 95

After the pressure treatment, the same coating composition as above, or a similar one, is then applied to both sides of the coated web in sufficient thickness to give a total coating composition weight of about 1.5 ounces per square 100 yard on each side. This second coating may also be applied in any conventional manner, the doctor knife being preferred.

A shade cloth thus prepared is of the so-called 105 translucent type and is of greatly improved appearance as compared with shade cloth as heretofore made, in which no pressure treatment is given to the cloth prior to application of the final coat of the coating composition. Due to the pressure treatment, the cloth is appreciably 110

improved with respect to the uniformity of translucency and clearness when viewed by transmitted light, two properties of the greatest importance when the appearance of shade cloth 5 is considered.

*Example 2.*—Shade cloth was prepared according to the method set forth in Example 1, except that the coating composition had the following formula:

|                 | Parts |
|-----------------|-------|
| Cellulose ester | 22-40 |
| Softener        | 15-30 |
| Pigment         | 35-40 |

15 The preferred composition in this example was:

|                 | Parts |
|-----------------|-------|
| Cellulose ester | 31    |
| Softener        | 23    |
| Pigment         | 46    |

20 The shade cloth prepared according to this example is similar to that obtained proceeding as in Example 1, except that the shade cloth is of the so-called opaque type, although it is 25 to be understood that the shade cloth is by no means absolutely opaque.

30 The particular cellulose ester coating composition used in the present method, both before and after the pressure treatment, may be varied widely and need not differ from such compositions heretofore used in this art. Generally, cellulose nitrate is the preferred cellulose ester, although cellulose acetate or other esters may be used. A 35 wide variety of softeners is available for these compositions, as is well known in the art. Among those most suitable are raw castor oil, blown castor oil, blown cottonseed or rapeseed oil, among the vegetable oil softeners, and the so-called solvent softeners such as dibutyl phthalate, dibutyl 40 tartrate, ethyl tartrate, and the like. Obviously, the choice of pigments is extremely wide and includes those commonly used in the industry, or combinations of several pigments, depending upon the translucency and color of the shade 45 cloth desired.

50 The improvement obtained in shade cloth material by the present method is quite unexpected, as the pressure treatment on the partially coated shade cloth not only securely anchors the coating composition in the cloth and thus improves the durability of the material, which might have been predicted by those acquainted with this art, but also improves the appearance of the shade 55 cloth to a remarkable degree, increasing the uniformity of the translucency of the cloth beyond expectation, and also giving the cloth greater clearness when viewed by transmitted light.

60 Although the present invention has been described as related to shade cloth, it will be apparent that the invention applies to other types of cellulose ester coated fabrics and the term "shade cloth" as used herein and in the appended claims is intended to include cellulose ester coated fabrics in general having properties similar to shade 65 cloth.

65 As many apparently widely different embodiments of this invention may be made without departing from the spirit and scope thereof, it is to be understood that we do not limit ourselves 70 to the specific embodiments thereof except as defined in the appended claims.

We claim:

75 1. Method of preparing shade cloth comprising applying 0.2-0.8 ounces per square yard of a coating composition including nitrocellulose, a softener

er and a pigment, to each side of a web of fabric, applying pressure to both sides of the coated web while the coatings are still in a plastic state, and then applying 0.7-1.3 ounces per square yard of a similar coating composition to each side of the 80 coated web.

2. Method of preparing shade cloth comprising applying 0.2-0.8 ounces per square yard of a coating composition including nitrocellulose, a softener and a pigment, to each side of a web of sheeting, applying pressure to both sides of the coated web while the coatings are still in a plastic state by running the coated web through a plate press or pressure rolls, and then applying 0.7-1.3 ounces per square yard of a similar coating composition 85 to both sides of the web.

3. Method of preparing shade cloth comprising applying 0.2-0.8 ounces per square yard of a coating composition including nitrocellulose, a softener, and a pigment, to each side of a web of fabric, applying pressure to both sides of the coated web while the coatings are still in a plastic state by 90 running the coated web through a plate press or pressure rolls, and then applying a similar coating composition to each side of the coated web.

4. Method of preparing shade cloth comprising applying 0.2-0.8 ounces per square yard of a coating composition including nitrocellulose, a softener, and a pigment, to each side of a web of fabric, applying pressure to both sides of the coated web while the coatings are still in a plastic state by 100 running the coated web through a plate press or pressure rolls, and then applying a similar coating composition to each side of the coated web.

5. Method of preparing shade cloth comprising applying 0.2-0.8 ounces per square yard of a coating composition including nitrocellulose, a softener, and a pigment, to each side of a web of fabric, applying a pressure of about 575 pounds per square inch to both sides of the coated web while the coatings are still in a plastic state by 110 running the coated web through a plate press or pressure rolls, and then applying a similar coating composition to each side of the coated web.

6. Method of preparing shade cloth comprising applying 0.2-0.8 ounces per square yard of a coating composition including nitrocellulose, a softener, and a pigment, to each side of a web of sheeting, applying a pressure of about 575 pounds per square inch to both sides of the coated fabric while the coatings are still in a plastic state by 120 running the coated web through a plate press or pressure rolls, and then applying 0.7-1.3 ounces per square yard of a similar coating composition to both sides of the web.

7. Shade cloth of uniform translucency comprising a fabric having a cellulose ester coating superposed on both sides of the fabric, said fabric having been coated with from 0.2-0.8 ounces per square yard of a coating composition comprising a cellulose ester, a softener, and a pigment, on both sides thereof, then subjected to pressure on both sides while the coatings were still in plastic state, and then further coated with a similar coating composition on both sides.

8. Shade cloth of uniform translucency comprising a fabric having a cellulose ester coating superposed on both sides of the fabric, said fabric having been coated with from 0.2-0.8 ounces per square yard of a coating composition comprising nitrocellulose, a softener, and a pigment, on both 140 sides thereof, then subjected to pressure on both sides while the coatings were still in a plastic state by running the fabric through a plate press or pressure rolls, and then further coated with a similar coating composition on both sides.

|    |                                                                                                                                                                                                                                                                                                                                                                                                                                                                                                                                                                                                                 |     |
|----|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----|
| 9. | Shade cloth of uniform translucency comprising a fabric having a cellulose ester coating superposed on both sides of the fabric, said fabric having been coated with from 0.2-0.8 ounces per square yard of a coating composition comprising a cellulose ester, a softener, and a pigment, on both sides thereof, then subjected to pressure on both sides while the coatings were still in a plastic state by running the fabric through a plate press or pressure rolls, and then further coated with from 0.7-1.3 ounces per square yard of a similar coating composition on each side of the coated fabric. | 80  |
| 10 | Shade cloth of uniform translucency comprising a fabric having a cellulose ester coating superposed on both sides of the fabric, said fabric                                                                                                                                                                                                                                                                                                                                                                                                                                                                    | 85  |
| 15 |                                                                                                                                                                                                                                                                                                                                                                                                                                                                                                                                                                                                                 | 90  |
| 20 |                                                                                                                                                                                                                                                                                                                                                                                                                                                                                                                                                                                                                 | 95  |
| 25 |                                                                                                                                                                                                                                                                                                                                                                                                                                                                                                                                                                                                                 | 100 |
| 30 |                                                                                                                                                                                                                                                                                                                                                                                                                                                                                                                                                                                                                 | 105 |
| 35 |                                                                                                                                                                                                                                                                                                                                                                                                                                                                                                                                                                                                                 | 110 |
| 40 |                                                                                                                                                                                                                                                                                                                                                                                                                                                                                                                                                                                                                 | 115 |
| 45 |                                                                                                                                                                                                                                                                                                                                                                                                                                                                                                                                                                                                                 | 120 |
| 50 |                                                                                                                                                                                                                                                                                                                                                                                                                                                                                                                                                                                                                 | 125 |
| 55 |                                                                                                                                                                                                                                                                                                                                                                                                                                                                                                                                                                                                                 | 130 |
| 60 |                                                                                                                                                                                                                                                                                                                                                                                                                                                                                                                                                                                                                 | 135 |
| 65 |                                                                                                                                                                                                                                                                                                                                                                                                                                                                                                                                                                                                                 | 140 |
| 70 |                                                                                                                                                                                                                                                                                                                                                                                                                                                                                                                                                                                                                 | 145 |
| 75 |                                                                                                                                                                                                                                                                                                                                                                                                                                                                                                                                                                                                                 | 150 |

CORNELIUS A. ALT.  
HERMAN C. GRAEBNER.  
LANCELOT MOFFETT.